

1

2,979,374

## FIBROUS TEXTILE CELLULOSIC PHOSPHONOMETHYL ETHERS AND PROCESS OF PREPARATION

George L. Drake, Jr., and Wilson A. Reeves, Metairie, and John D. Guthrie, New Orleans, La., assignors to the United States of America as represented by the Secretary of Agriculture

No Drawing. Filed Oct. 31, 1957, Ser. No. 693,787

4 Claims. (Cl. 8—120)

(Granted under Title 35, U.S. Code (1952), sec. 266)

A non-exclusive, irrevocable, royalty-free license in the invention herein described, throughout the world for all purposes of the United States Government, with the power to grant sublicenses for such purposes, is hereby granted to the Government of the United States of America.

This invention relates to the ethers of fibrous cellulose in which the fibrous form and the properties it produces in textiles, i.e., properties such as hand, feel, tensile strength and the like are retained substantially unaltered or with proper degree of substitution can change all of these properties with the formation of a water-soluble cellulosic material. This invention provides fibrous phosphonomethyl ethers of cellulose; the salts of such ethers; soluble phosphonomethyl ethers of cellulose; a process of reducing the combustibility of fibrous cellulosic materials; and a process of producing fibrous cellulose with high cation exchange capacity.

It is known that 2-phosphatoethyl ethers of cellulose can be made. For example, Leon H. Chance et al. in United States Patent 2,743,232, dated April 24, 1956, had demonstrated that fibrous 2-phosphatoethyl ethers of cellulose can be produced by reacting a cellulosic material with 2-chloroethylphosphoric acid in aqueous alkali. In that patent he converted the hydroxyl groups of the cellulose material to 2-phosphatoethyl groups



In his invention he introduced a group into the cellulosic molecule in which the phosphorus is joined to the carbon through an oxygen atom which is an ester linkage. We have found that we can convert the hydroxyl group of the cellulose material to phosphonomethyl groups  $(-\text{OCH}_2\text{PO}_3=)$ . In this case the phosphorus is joined to the carbon atom directly and the linkage between the phosphonomethyl group and the cellulose is an ether linkage. Since this is an ether linkage it should be a more stable link since it is generally known that esters are subject to acid and basic hydrolysis whereas ethers are not. It is reported in the literature [M. I. Kabachnik and T. Ya. Medved, Izvest. Akad. Nauk S.S.R., Otdel. Khim. Nauk 1951, 95-7; M. I. Kabachnik, E. S. Shepeleva, Izvest. Akad. Nauk S.S.R., Otdel. Khim. Nauk 1951, 185-91] that the reactivity of the halogen atom on the compound with the structure



or its derivative is very low so that the  $\text{PO}_3$  grouping may be said to be passivating rather than activating. It

2

is surprising, therefore, that contrary to this fact, we have now found that using the proper conditions we can make this halogen react with the hydroxyls of a cellulosic material in the presence of an alkali metal hydroxide even without the use of pressure. We have also found that with proper conditions a water soluble derivative of a cellulose can be obtained.

It is an object of our invention to provide new fibrous metal salts of phosphonomethyl ethers of cellulose. Another object is to produce a new water soluble phosphonomethyl ether of cellulose. Another object is to produce a new fibrous phosphonomethyl ether of cellulose which has a high cation exchange capacity. Another object is to provide a process of reducing the combustibility of fibrous cellulosic materials. Other objects will become apparent hereinafter.

In accordance with the invention we prepare this new phosphonomethyl ether of cellulose by reacting a fibrous cellulosic material containing hydroxyl groups with an aqueous solution of an alkali metal salt of chloromethyl phosphonic acid (or other salts of the acid in which the alkali metal will replace the cations of the salt) and an excess of alkali metal hydroxide. The corresponding phosphonic acid derivative of cellulose can be produced by soaking the phosphonomethyl ether of cellulose in a dilute aqueous solution of a strong mineral acid until all of the alkali metal atoms have been replaced by hydrogen atoms.

Reduction of the combustibility of fibrous cellulosic materials containing hydroxyl groups is produced by converting the phosphonomethyl ether of cellulose to the corresponding free acid derivative in the above way and converting this derivative to the corresponding ammonium salt by reacting with ammonia.

Soluble fibrous phosphonomethyl cellulose is produced by allowing a cellulosic material containing hydroxyl groups to be wet out with a solution consisting of an alkali metal salt of chloromethyl phosphonic acid and excess alkali metal hydroxide dissolved in water, at a temperature which is sufficient to convert the hydroxyl groups of the cellulosic material to phosphonomethyl groups  $(-\text{OCH}_2\text{PO}_3=)$  where the order of substitution is such that 2% or more phosphorus is introduced.

Cotton fibers, regenerated cotton fibers, aminated cotton fibers, carboxymethylated cotton fibers, paper, sulfonated cotton fibers, and other like materials containing one or more hydroxyl groups per anhydroglucoside unit are suitable fibrous cellulosic materials. Cotton fiber is the preferred material. The above disclosed reactions can also be extended to cover other types of polysaccharide hydroxyls for example starch, sugar and any material containing one or more hydroxyls per anhydroglucoside unit.

Free fibers, sliver, yarn or fabric can be phosphonomethylated, but yarn or fabric is preferred.

Phosphonomethyl groups can be introduced into cellulosic materials by using the metal salt of the chloromethyl phosphonic acid, or the acid chloride. The metal salt is preferred. This invention is not limited to the chloroderivative. Compounds having the following structure are suitable:

65



70 where X is any of the halogens and R is hydrogen, alkyl, aryl, alkyl-aryl or substituted alkyl, aryl or alkyl-aryl groups.

The aqueous solution suitable for use in the present process can be aqueous solutions of the salt and any alkali metal hydroxide containing from about 10% to 30% by weight of unreacted alkali metal hydroxide and from about 1% to 30% by weight of the alkali metal salt of chloromethyl phosphonic acid. Aqueous solutions containing from about 20% to 30% unreacted sodium hydroxide and from 12% to 15% of the sodium salt of the acid are preferred.

A variety of ways can be used to produce the fibrous phosphonomethyl ethers of cellulose. The cellulosic material can be wet out by either of the aqueous solutions first followed by the other, or by wetting out the material using an aqueous solution containing a mixture of the two salts such that the required concentration of salts necessary for the introduction of the phosphonomethyl groups are present. The one solution method is preferred.

The reaction can be conducted at temperatures from about 20° C. to temperatures at which the thermal decomposition of the cellulosic material becomes noticeable. Preferably cotton fabric is padded with an aqueous solution containing chloromethyl phosphonic acid disodium salt and unreacted sodium hydroxide to a pickup of around 125-200% and heating from about 75-115° C. for about 5 to 30 minutes or from about 2 to 10 minutes at about 140° to 160° C.

The impregnated fibrous cellulosic material can be heated using any conventional heating apparatus; for example, ovens, hot boxes, heated cans, heated tenter frame, molten metal bath, infrared lamps, lens and sunlight, irons, presses and the like. Excess salts are washed free from the fibrous cellulosic material with water or a water-alcohol mixture and dried by any of the above heating equipment.

The combustibility of the fibrous cellulosic material, preferably cotton, is reduced by phosphonomethylating to a phosphorus content of about 0.2%. Higher contents can be obtained using the proper conditions. The alkali metal salts can be converted to the dibasic acid and then converted to the ammonium salt and with values of about 0.2% phosphorus will produce a black char on burning with no afterglow. Even with such a small add-on this process could be used in aiding other flame retardants where afterglow is a problem or where a tough ash is needed. The ammonium salts of phosphonomethylated fibrous cellulosic material containing about 1 to 3% phosphorus will not burn even if a small strip is held in the vertical position and lighted at the bottom.

Water soluble cellulosic materials can be obtained by wetting the cellulosic material with an aqueous solution consisting of about 20 to 25% NaOH and about 10 to 20% chloromethyl phosphonic acid and heating from about 5 to 30 minutes at 120° to 150° C. Water solubility can be obtained using fibers, yarn or fabric. For example, varying amounts of substitution are necessary dependent on the form of cellulosic material used. Two percent phosphorus on cellulosic yarn is readily soluble in 1% alkali or water. Washing of the soluble yarn is best done using alcohol-water mixtures varying in alcohol content from about 2% to about 80%. The preferred amount is about 20 to 40%. The soluble phosphonomethylated cellulosic material can be reprecipitated in alcohol, acetone and other similar solvents. This offers the possibility of making phosphorus containing fibers by extrusion. This water soluble derivative can be further used as a phosphorus containing size for other materials. Since this soluble phosphonomethylated cellulosic material contains reactive groups it is possible to form a permanent size containing phosphorus and also offer some flame retardancy.

The reactive phosphonomethyl groups of the phosphonomethylated cellulose react with ethylene oxide, ethyl-

eneimine or derivatives such as butadiene dioxide, tris 1-aziridinyl phosphine oxide or sulfide and the like and enhance the properties of the textile products such as flame retardancy, change the ion exchange capacity and also render the water soluble phosphonomethylated cellulose insoluble.

#### Combustibility tests

The fabric prepared in the following examples was cut into strips 1 cm. wide and at least 5 cm. long. The strips were held with their surface vertical and their long edge at the indicated angle from the vertical and ignited at the specified point. Whether or not the burning would continue along the strip and the presence or absence of afterglow was observed. Strips of the cloth used in each of the examples, prior to treatment, would burn continuously even when held vertically and ignited at the top.

#### EXAMPLE I

##### Phosphonomethylation

48 x 48 cotton sheeting fabric was padded using 2 dips and 2 nips and light squeeze roll pressure, with a solution consisting of: 15 parts chloromethyl phosphonic dichloride, 25 parts sodium hydroxide and 60 parts water. Solution wet pickup was 143%. The wet fabric was heated for 30 minutes at 110° C. in a forced draft oven, washed with water and dried. The cloth contained 1.99% phosphorus and had an ion exchange capacity of 1.179 meq./gm. A strip of the fabric would pass the 90° angle flame test with a slight afterglow.

##### Ammonium salt production

The regeneration of the ether sodium salt to the corresponding ammonium salt was made by soaking a sample of the cloth for 15 minutes in 5% hydrochloric acid, washed free of the acid with distilled water, then soaked in 5% ammonium hydroxide. This was washed with distilled water and dried. It now contained 1.95% phosphorus and 0.78% nitrogen. It would pass the standard vertical flame test and would pass the 180° angle strip test with no afterglow.

##### Preparation of the solution for Example I

Solution was made as follows: The specified amount of chloromethyl phosphonic dichloride was reacted (keeping the solution cool) with the calculated quantity of NaOH to form the sodium salt of the acid. The water used for the NaOH solution which was used to neutralize the acid chloride was taken from the total amount of water used in the preparation of the desired percent solution. This solution and the required quantity of unreacted NaOH and remaining water was cooled and then mixed.

#### EXAMPLE II

##### Curing times, curing temperature, caustic concentrations and chloromethyl phosphonic dichloride concentration in relation to phosphorus content

##### SOLUTIONS<sup>1</sup>

| Solution Number | Percent NaOH unreacted | Percent ClCH <sub>2</sub> POCl <sub>3</sub> | Percent H <sub>2</sub> O |
|-----------------|------------------------|---------------------------------------------|--------------------------|
| 1               | 10                     | 15                                          | 75                       |
| 2               | 10                     | 30                                          | 60                       |
| 3               | 25                     | 15                                          | 60                       |
| 4               | 25                     | 30                                          | 45                       |

<sup>1</sup> Solutions were prepared using procedure as in preparation in Example I.

Six pieces of 48 x 48 cotton sheeting were padded through each of the above solutions using 2 dips, 2 nips and a light squeeze roll setting. The cation exchange capacities, elemental analyses conditions and other data are listed in the following tables:

Fabrics were processed as in Example II.

SOLUTION 1

| 5  | Cure Temperature, °C. | Cure Time, min. | Percent Phosphorus | Cation Exchange Capacity, meq./gm. | Strip Burn Angle on NH <sub>4</sub> Salt, degrees |
|----|-----------------------|-----------------|--------------------|------------------------------------|---------------------------------------------------|
|    | 110.....              | 5               | 0.14               | 0.160                              | 0-black ash no after-glow.                        |
| 10 | 110.....              | 30              | 0.88               | 0.649                              | 135.                                              |
|    | 140.....              | 5               | 0.90               | 0.658                              | 135.                                              |
|    | 140.....              | 30              | 0.90               | 0.678                              | 135.                                              |

SOLUTION 1

| Cure Temperature, °C. | Cure Time   | Percent Phosphorus | Cation Exchange Capacity, meq./gm. | Strip Burn Angle on NH <sub>4</sub> Salt, degrees |
|-----------------------|-------------|--------------------|------------------------------------|---------------------------------------------------|
| Room temperature...   | 24 hrs..... | 0.02               | 0.063                              | 0-black ash no after-glow.                        |
| 110.....              | 5 min.....  | 0.02               | 0.055                              | Do.                                               |
| 110.....              | 30 min..... | 0.03               | 0.076                              | Do.                                               |
| 140.....              | 5 min.....  | 0.05               | 0.084                              | Do.                                               |
| 140.....              | 30 min..... | 0.13               | 0.122                              | Do.                                               |

SOLUTION 2

| Room temperature... | Cure Time   | Percent Phosphorus | Cation Exchange Capacity, meq./gm. | Strip Burn Angle on NH <sub>4</sub> Salt, degrees |
|---------------------|-------------|--------------------|------------------------------------|---------------------------------------------------|
| Room temperature... | 24 hrs..... | 0.02               | 0.073                              | 0-black ash no after-glow.                        |
| 110.....            | 5 min.....  | 0.03               | 0.062                              | Do.                                               |
| 110.....            | 30 min..... | 0.035              | 0.050                              | Do.                                               |
| 140.....            | 5 min.....  | 0.03               | 0.052                              | Do.                                               |
| 140.....            | 30 min..... | 0.10               | 0.096                              | Do.                                               |

SOLUTION 3

| Room temperature... | Cure Time   | Percent Phosphorus | Cation Exchange Capacity, meq./gm. | Strip Burn Angle on NH <sub>4</sub> Salt, degrees |
|---------------------|-------------|--------------------|------------------------------------|---------------------------------------------------|
| Room temperature... | 24 hrs..... | 0.02               | 0.100                              | 0-black ash no after-glow.                        |
| 110.....            | 5 min.....  | 1.54               | 0.975                              | 160.                                              |
| 110.....            | 30 min..... | 1.82               | 1.184                              | 180.                                              |
| 140.....            | 5 min.....  | 1.99               | 1.284                              | 180.                                              |
| 140.....            | 30 min..... | 1.96               | 1.286                              | 180.                                              |

SOLUTION 4

| Cure Temperature, °C. | Cure Time, min. | Percent Phosphorus | Cation Exchange Capacity, meq./gm. | Strip Burn Angle on NH <sub>4</sub> Salt, degrees | NH <sub>4</sub> Salt |           |
|-----------------------|-----------------|--------------------|------------------------------------|---------------------------------------------------|----------------------|-----------|
|                       |                 |                    |                                    |                                                   | Percent P            | Percent N |
| 110.....              | 5               | 0.94               | 0.621                              | 160                                               | -----                | -----     |
| 110.....              | 30              | 1.60               | 0.992                              | 180                                               | -----                | -----     |
| 140.....              | 5               | 1.78               | 1.107                              | 180                                               | -----                | -----     |
| 140.....              | 30              | 1.46               | 0.928                              | 180                                               | 1.45                 | 0.60      |

EXAMPLE III

Curing times and temperatures keeping caustic concentration constant and varying  $\text{ClCH}_2\text{POCl}_2$  concentration in relation to phosphorus content

SOLUTIONS 1

| Solution Number | Percent NaOH unreacted | Percent $\text{ClCH}_2\text{POCl}_2$ | Percent H <sub>2</sub> O |
|-----------------|------------------------|--------------------------------------|--------------------------|
| 1.....          | 25                     | 5                                    | 70                       |
| 2.....          | 25                     | 10                                   | 65                       |
| 3.....          | 25                     | 15                                   | 60                       |
| 4.....          | 25                     | 30                                   | 45                       |

SOLUTIONS

| 65 | Solution Number | Percent NaOH unreacted | Percent $\text{ClCH}_2\text{POCl}_2$ | Percent H <sub>2</sub> O |
|----|-----------------|------------------------|--------------------------------------|--------------------------|
|    | 1.....          | 25                     | 2                                    | 73                       |
|    | 2.....          | 25                     | 5                                    | 70                       |
|    | 3.....          | 25                     | 10                                   | 65                       |
| 70 | 4.....          | 25                     | 15                                   | 60                       |

48 x 48 cotton sheeting was treated as in Example I.  
75 A wet pickup of 173% was obtained.

<sup>1</sup> Solutions were made using the same procedure as in Example I.

## SOLUTION 1

| Cure Temperature, °C. | Cure Time | Percent Phosphorus | Cation Exchange Capacity, meq./gm. | Strip Burn Angle on NH <sub>4</sub> Salt, degrees | NH <sub>4</sub> Salt |           |
|-----------------------|-----------|--------------------|------------------------------------|---------------------------------------------------|----------------------|-----------|
|                       |           |                    |                                    |                                                   | Percent P            | Percent N |
| 110                   | 5 min     | 0.36               | 0.300                              | 45                                                | 0.30                 | 0.13      |
| 110                   | 30 min    | 0.44               | 0.342                              | 90                                                |                      |           |
| 140                   | 5 min     | 0.42               | 0.329                              | 100                                               |                      |           |
| 140                   | 30 min    | 0.42               | 0.360                              | 110                                               |                      |           |
| Room temperature      | 18 hrs    | 0.015              | 0.073                              | 0-black ash no after-glow.                        |                      |           |

## SOLUTION 2

| Cure Temperature, °C. | Cure Time | Percent Phosphorus | Cation Exchange Capacity, meq./gm. | Strip Burn Angle on NH <sub>4</sub> Salt, degrees |
|-----------------------|-----------|--------------------|------------------------------------|---------------------------------------------------|
| 110                   | 5 min     | 0.15               | 0.166                              | 0-black ash no after-glow.                        |
| 110                   | 30 min    | 0.76               | 0.574                              | 135                                               |
| 140                   | 5 min     | 0.81               | 0.570                              | 135                                               |
| 140                   | 30 min    | 0.87               | 0.584                              | 135                                               |
| Room temperature      | 18 hrs    | 0.015              | 0.063                              | 0-black ash no after-glow.                        |

## SOLUTION 3

| Cure Temperature, °C. | Cure Time | Percent Phosphorus | Cation Exchange Capacity, meq./gm. | Strip Burn Angle on NH <sub>4</sub> Salt, degrees | NH <sub>4</sub> Salt |           |
|-----------------------|-----------|--------------------|------------------------------------|---------------------------------------------------|----------------------|-----------|
|                       |           |                    |                                    |                                                   | Percent P            | Percent N |
| 110                   | 5 min     | 0.92               | 0.594                              | 90                                                | 0.74                 | 0.38      |
| 110                   | 30 min    | 1.72               | 1.110                              | 175                                               |                      |           |
| 140                   | 5 min     | 1.62               | 1.070                              | 175                                               |                      |           |
| 140                   | 30 min    | 1.50               | 1.000                              | 140                                               |                      |           |
| Room temperature      | 18 hrs    | 0.01               | 0.073                              | 0-black ash no after-glow.                        |                      |           |

## SOLUTION 4

|     |    |      |       |     |      |      |
|-----|----|------|-------|-----|------|------|
| 110 | 5  | 2.0  | 1.312 | 180 | 2.01 | 0.85 |
| 110 | 30 | 2.25 | 1.446 | 180 |      |      |
| 140 | 5  | 2.23 | 1.403 | 180 |      |      |
| 140 | 30 | (1)  |       |     |      |      |

1 Dissolved.

## EXAMPLE V

## Phosphonomethylation of aminized cotton fabric

A sample of aminized 48 x 48 cotton sheeting containing 0.7% nitrogen was padded with a solution composed of 25% NaOH, 15%



and 60% water using 2 dips and 2 nips with a light squeeze roll pressure. The wet sample was heated in a forced draft oven for 30 minutes at 140° C. A good reaction was obtained. The fabric was slimy when wet and had a leather-like feel when wet. When dry it was parchment like. It would pass the 90-110 angle flame test not in the ammonium salt form.

## EXAMPLE VI

## Phosphonomethylation of cotton in yarn form to produce water soluble cotton

12-4's cotton yarn which had been scoured, bleached

and mercerized was padded with a solution consisting of 35.1 parts by weight



96.5 parts by weight of NaOH and 180 parts by weight of water to a wet pickup of 196%. Heated for 30 minutes at 140° C. and washed in 20% ethanol-water solution. Dried. The yarn had a weight increase of 13%. A sample of this yarn when placed in water dissolved immediately. The phosphorus content was 2.12%. The yarn would pass the 90°-110° strip burn angle test in the sodium salt form. In the ammonium salt form the yarn could not be ignited.

15

## Example VII

The same solution and procedure used in Example VI was repeated on 48 x 48 cotton sheeting. It was also water soluble and contained 2.4% phosphorus. It took longer to go into solution than the yarn sample in Example VI. The flammability was the equivalent of the yarn in Example VI.

25

EXAMPLE VIII  
pH in relation to cation exchange capacity of phosphonomethylated cotton

48 x 48 cotton sheeting was padded through solution 4 of Example IV using 2 dips and 2 nips with a light squeeze roll pressure to a wet pickup of 143.3%. The sample was cured for 30 minutes in an oven at 110° C. The sample was washed and dried. The sample contained 2.0% phosphorus and had a cation exchange capacity of 1.180 meq./gm.

35

## pH VS. CAPACITY

| pH    | Cation Exchange Capacity, meq./gm. |
|-------|------------------------------------|
| 1.60  | 0.2067                             |
| 1.92  | 0.2980                             |
| 2.10  | 0.3466                             |
| 2.38  | 0.4149                             |
| 3.54  | 0.5549                             |
| 5.97  | 0.6199                             |
| 6.64  | 0.7114                             |
| 7.03  | 0.8159                             |
| 7.38  | 0.9150                             |
| 8.59  | 1.0290                             |
| 11.44 | 1.3229                             |
| 11.73 | 1.4455                             |

45

## EXAMPLE IX

## Repeated phosphonomethylation

48 x 48 cotton sheeting was padded through a solution containing 25% unreacted caustic and 15% chloromethyl phosphonic dichloride (converted to the sodium salt by hydrolysis with the calculated quantity of water and then to the sodium salt by adding the calculated quantity of sodium hydroxide) and 60% water. The wet fabric was heated in a forced draft oven for 30 minutes at 140° C., washed and dried. The phosphorus content was 1.84% and the cation exchange capacity was 1.075 meq./gm. The angle strip burn ammonium salt form was 180°. This fabric was retreated in the above manner. It had a phosphorus content of 3.96% and a cation exchange capacity of 2.333 meq./gm. The ammonium salt form could not be ignited.

We claim:

1. A process for preparing chemically modified fibrous cellulosic textile material containing from about 0.02% to about 5.0% phosphorus in the form of phosphono-methyl ether of cellulose comprising: padding a fibrous cellulosic textile material having at least one free hydroxyl group per anhydroglucoside unit of the cellulose

50

75

molecule with an aqueous solution containing from 5 to 20% by weight of an alkali metal salt of chloromethyl phosphonic acid and 15 to 25% by weight of an alkali metal hydroxide to a wet pickup of from 125 to 200%, heating the padded fibrous cellulosic textile material for from 5 to 30 minutes at temperatures of from 16 to 140° C., the higher temperatures being used with the shorter heating times.

2. A process for reducing the combustibility of fibrous cellulosic textile materials comprising: wetting textile fibers having at least one free hydroxyl group per anhydroglucose unit of the cellulose molecule with an aqueous solution containing from 5 to 15% by weight of an alkali metal salt of chloromethyl phosphonic acid and from 15 to 25% by weight of an alkali metal hydroxide to a wet pickup of from 125 to 200%, heating the wetted textile material for from 5 to 30 minutes at a temperature of from 60 to 140° C., employing the shorter times with the higher temperatures, rinsing the heated textile material free of alkali with a 1 to 5% aqueous solution of a strong mineral acid, rinsing the acid-treated textile material in water, and then neutralizing the acid-treated tex-

5

10

tile material with a 5% aqueous solution of ammonium hydroxide.

3. A chemically modified cellulosic textile in which some of the hydroxyl groups have been converted to  $-\text{OCH}_2\text{PO}_3\text{X}_2$  groups in which X is a member of the group consisting of hydrogen, alkali metal, and  $\text{NH}_4$ , the degree of conversion being such that the modified cellulosic textile contains from 0.01% to 4.0% by weight of the modified cellulosic textile of phosphorus.

15

15

4. A chemically modified water soluble cotton textile in which some of the hydroxyl groups have been converted to  $-\text{OCH}_2\text{PO}_3\text{X}_2$  groups in which X is a member of the group consisting of hydrogen, alkali metal, and  $\text{NH}_4$ , wherein the degree of conversion is such that the modified cotton contains from 2.0% to 4.0% by weight of the modified cotton of phosphorus.

## References Cited in the file of this patent

## UNITED STATES PATENTS

|           |            |               |
|-----------|------------|---------------|
| 2,743,232 | Chance     | Apr. 24, 1950 |
| 2,678,330 | Van Gorder | May 11, 1954  |
| 2,691,567 | Kvalnes    | Oct. 12, 1954 |